

## UNITED STATES PATENT OFFICE

2,374,563

## STABILIZED DIAZO-TYPE SENSITIVE MATERIAL

Maximilian K. Reichel, Albany, N. Y., assignor to  
General Aniline & Film Corporation, New York,  
N. Y., a corporation of Delaware

No Drawing. Application December 4, 1942,  
Serial No. 467,902

13 Claims. (Cl. 95—6)

This invention relates to the stabilization of light-sensitive layers which are produced by the incorporation of a diazo compound as the light-sensitive medium onto the surface of a suitable carrier base. More particularly, it refers to the stabilization of so-called dry development diazo-type light-sensitive layers wherein the diazo compound is a diazo compound derived from ortho or para aminonaphthol or from N-mono or di-substituted aromatic para-diamines, which diazo compound is incorporated into the light-sensitive layer, together with an azo dyestuff coupling component.

Various processes are known for the preparation of light-sensitive layers which depend upon the use of a diazo compound as the light-sensitive medium, and various materials have been employed for the carrier of the light-sensitive layer, including textiles, paper, cellulosic films, and glass and metal surfaces. The sensitized carrier is exposed to light under a transparent original which it is desired to reproduce and the diazo compound is decomposed in the areas unprotected by the outline of the original. The undecomposed diazo compound in the protected areas is then used to develop the image of the original by coupling the said diazo compound in alkaline atmosphere, with an azo dyestuff coupling component. In the two component layers which contemplate the incorporation of the coupling component into the light-sensitive layer with the diazo compound, the development of the dyestuff forming the image is effected by bringing the exposed light-sensitive layer into contact with ammonia gas. This is known as the dry developing process.

The dyestuff components, as applied on the carrier, are relatively unstable and cannot be stored for long periods prior to use. The light-sensitive layers which carry the coupling component as well as the diazo compound in the light-sensitive layer are subject to premature coupling of the said dyestuff components as well as decomposition of the diazo compound upon long storage. Many attempts have been made to obtain more stable coating solutions and to render the light-sensitive layers produced therefrom less sensitive to deterioration without impairing the light-sensitive qualities of the diazo compound upon which the production of accu-

rate images from the original depends. These attempts have hitherto been relatively unsuccessful. It is therefore the object of this invention to provide coating solutions and light-sensitive layers, using diazo compounds as the light-sensitive medium which can be stored for long periods prior to use and will be stable during storage even under unfavorable conditions.

I have found that coating solutions and the light-sensitive layers prepared therefrom can be stabilized against decomposition of the light-sensitive material and premature coupling of the dyestuff components by adding to the coating solution a compound of the following class: saturated and unsaturated gamma lactones of the following general formulae:



and

40

45

wherein X is a member of the group consisting of H, OH, COOH and alkyl, Y is a member of the group consisting of H and alkyl, Z is a member of the group consisting of H and OH, R is a lower alkyl radical, R<sub>1</sub> is a member of the group

consisting of H and COOH, and Alk means alkylene.

Examples of such compounds are:

1. Gamma-valero lactone



2. Gamma-valero lactone  $\gamma$ -carbonic acid



3.  $\gamma$ -Dihydroxy lactone of the gamma-hydroxy crotonic acid



4.  $\gamma$ -Dihydroxy lactone of the gamma-hydroxy  $\beta$ -methyl crotonic acid



5.  $\alpha$ -Angelica lactone



6.  $\beta$ -Angelica lactone



Diazotype light-sensitive layers which have been stabilized by addition of the gamma lactones of the above class show greatly improved keeping qualities and are stable against decomposition or deterioration for much longer periods of storage than hitherto possible when using the same diazo light-sensitive compositions without the gamma lactone stabilizers. The following examples illustrate the invention but they are not intended to limit it thereto. The parts are by weight unless otherwise stated.

Example I

|                                               |                 |      |    |
|-----------------------------------------------|-----------------|------|----|
| 2.1-diazo-hydroxy-naphthalene-5 sulfonic acid | parts           | 14.0 | 70 |
| Concentrated hydrochloric acid                | parts by volume | 7.0  |    |
| Nickel sulphate                               | parts           | 31.5 |    |
| Phloroglucine                                 | do              | 4.9  |    |
| Thiourea                                      | do              | 20.0 | 75 |

are dissolved in 1000 cc. of water. To this coating solution there are added 10.2 grams of gamma valero lactone per liter. This solution is then spread on paper, fabric, film or the like by the usual coating method for the production of diazo type light-sensitive layers, using a doctor blade to insure a thin even coating.

After storage at room temperature for several months, the stability of the sensitized material containing the gamma valero lactone was tested by exposing a test piece to light under a suitable diapositive and developing the image by application of ammonia gas. The resulting image reproduced on the light-sensitive layer containing the gamma valero lactone was compared with the image reproduced under the same conditions on a light-sensitive layer made from the same coating composition but containing no gamma valero lactone which latter had been stored under the same conditions for the same length of time. The background and consequently the contrast of the image reproduced on the light-sensitive layer made in accordance with this example is superior to that of the sample which does not contain the gamma valero lactone in the light-sensitive layer.

Example II

The composition of the coating solution is the same as in Example I but as a stabilizer 13.4 grams of gamma valero lactone  $\gamma$  carbonic acid per liter are used instead of the gamma valero lactone. The coating, storage and testing procedures are the same as in Example I. The stability of the coating made according to this example was found to be superior to that of a coating made from a solution not containing a gamma lactone stabilizer.

40

The composition of the coating solution is the same as in Example I but as a stabilizer 10.4 grams of the  $\gamma$  di-hydroxy lactone of gamma-hydroxy crotonic acid per liter are used instead of the gamma valero lactone. The coating, storage and testing procedures are the same as in Example I. The stability of the coating made according to this example was found to be superior to that of a coating made from a solution not containing a gamma lactone stabilizer.

Example III

The composition of the coating solution is the same as in Example I but as a stabilizer 11.8 grams of the  $\gamma$  di-hydroxy lactone of gamma-hydroxy betamethyl crotonic acid per liter are used instead of the gamma valero lactone. The coating, storage and testing procedures are the same as in Example I. The stability of the coating made according to this example was found to be superior to that of a coating made from a solution not containing a gamma lactone stabilizer.

Example IV

The composition of the coating solution is the same as in Example I but as a stabilizer 8.7 grams of alpha-beta-angelica lactone are used instead of the gamma valero lactone. The coating, storage and testing procedures are the same as in Example I. The stability of the coating made according to this example was found to be superior to that of a coating made from a solution not containing a gamma lactone stabilizer.

Example V

*Example VI*

|                                                                                                    | Parts |
|----------------------------------------------------------------------------------------------------|-------|
| Zinc chloride double salt of the diazo-compound obtained from N-ethanol-ethyl amino-4-aminobenzene | 10.5  |
| Citric acid                                                                                        | 50.0  |
| 2,3-dihydroxy-naphthalene                                                                          | 5.9   |
| Thiourea                                                                                           | 45.0  |
| The sodium salt of the naphthalene-1,3,6-trisulfonic acid                                          | 32.5  |
| Aluminum sulphate                                                                                  | 6.9   |

are dissolved in 1000 cc. of water. To this solution there are added 10.2 grams of gamma valero lactone per liter. The solution is then spread on a suitable base, such as paper, fabric, film or the like by the usual coating method in the same manner as described in Example I. The light-sensitive layer thus produced is then stored at room temperature for several months and its stability is then tested by observing the appearance of color in the light-sensitive layer due to premature coupling of the dye components and by comparison of its light-sensitive qualities with those of a test sample prepared and treated in the same manner as the light-sensitive layer of this example but omitting the gamma valero lactone stabilizer. When so tested, it was found that the light-sensitive layers made in accordance with this example show a negligible amount of coloring due to premature coupling of the dye components after the storage period, whereas, light-sensitive layers made from the same solution but not having the gamma valero lactone stabilizing agent, under the same conditions, show a considerable amount of coloring due to premature coupling. It also was found that upon exposure to light under a suitable diapositive and development of the image by application of ammonia gas, the light-sensitive layers of this example produce images having better definition and less background color than do light-sensitive layers not having the gamma valero lactone stabilizing agent, but otherwise having been made and treated the same as the light-sensitive layers of this example.

*Example VII*

The composition of the coating solution is the same as in Example VI but as a stabilizer 13.4 grams of gamma valero lactone  $\gamma$  carbonic acid per liter are used instead of the gamma valero lactone. The coating, storage and testing procedures are the same as in Example VI. The stability of the coating made according to this example was found to be superior to that of a coating made from a solution not containing a gamma lactone stabilizer.

*Example VIII*

The coating composition is the same as in Example VI but as a stabilizer 10.4 grams of the di-hydroxy lactone of gamma-hydroxy crotonic acid per liter are used instead of the gamma valero lactone. The coating, storage and testing procedures are the same as in Example VI. The stability of the coating made according to this example was found to be superior to that of a coating made from a solution not containing a gamma lactone stabilizer.

*Example IX*

The coating composition is the same as in Example VI but as a stabilizer 11.8 grams of the  $\gamma$  di-hydroxy lactone of gamma-hydroxy beta-methyl crotonic acid per liter are used instead

of the gamma valero lactone. The coating, storage and testing procedures are the same as in Example VI. The stability of the coating made according to this example was found to be superior to that of a coating made from a solution not containing a gamma lactone stabilizer.

*Example X*

The composition of the coating solution is the same as in Example VI but as a stabilizer 8.7 grams of alpha-beta-angelica lactone per liter are used instead of the gamma valero lactone. The coating, storage and testing procedures are the same as in Example VI. The stability of the coating made according to this example was found to be superior to that of a coating made from a solution not containing a gamma lactone stabilizer.

Various changes may be made in the details of my invention as described in the foregoing specification within the scope of the claims appended hereto without sacrificing the advantages of my invention.

*Example XI*

|                                                                                                          | Parts |
|----------------------------------------------------------------------------------------------------------|-------|
| Zinc chloride double salt of the diazo-compound obtained from N-mono-ethyl-amino-2-methyl-4-aminobenzene | 9.8   |
| Citric acid                                                                                              | 50    |
| 2,3-dihydroxy-naphthalene                                                                                | 5.9   |
| Thiourea                                                                                                 | 45    |
| The sodium salt of the naphthalene-1,3,6-trisulfonic acid                                                | 32.5  |
| Aluminum sulfate are dissolved in 1000 cc. of water                                                      | 6.9   |

To this solution there are added 10.2 grams of gamma valero lactone per liter. The coating, storage and testing procedures are the same as in Example I. The stability of the coating made according to this example was found to be superior to that of a coating made from a solution not containing a gamma lactone stabilizer.

*Example XII*

|                                                                                                    | Parts |
|----------------------------------------------------------------------------------------------------|-------|
| Zinc chloride double salt of the diazo-compound obtained from N-ethanol-ethyl-amino-4-aminobenzene | 10.5  |
| Citric acid                                                                                        | 5     |
| Thiourea                                                                                           | 45    |
| The sodium salt of the naphthalene-1,3,6-trisulfonic acid                                          | 32.5  |
| The aluminum sulfate are dissolved in 1000 cc. of water                                            | 6.9   |

To this solution there are added 10.2 grams of gamma valero lactone per liter. The solution is then spread on a suitable base, such as paper, fabric, film or the like by the usual coating method in the same manner as described in Example I. The light-sensitive layer thus produced is then stored at room temperature for several months and its stability is then tested by observing the appearance of color in the light-sensitive layer due to decomposition of the diazo-compound and by comparison with that of a test sample prepared and treated in the same manner as the light-sensitive layer of this example but omitting the gamma valero lactone. The test pieces are then exposed to light under a suitable diapositive and the images developed by application of an alkali solution of a suitable azo-component such as phloro-glucine, resorcin, or 2 - 3 - dihydroxy - naphthalene. The resulting image reproduced on the light-sensitive layer containing the gamma valero lactone showed a

higher color contrast of the image indicating the prevention of the decomposition and the consequent discoloration of the diazo-compound while at storage.

I claim:

1. The process of increasing the stability of a diazo-type light-sensitive layer containing a suitable diazo compound which comprises adding to the coating solution a member of the class consisting of saturated and unsaturated gamma lactones of the following formulae:



and



wherein X is a member of the group consisting of H, OH, COOH and alkyl, Y is a member of the group consisting of H and alkyl, Z is a member of the group consisting of H and OH, R is a lower alkyl radical, R1 is a member of the group consisting of H and COOH, and Alk means alkylene; and coating a suitable base with said solution.

2. The process of increasing the stability of a diazo-type light-sensitive layer containing a diazo compound suitable for forming a stable two component diazotype layer and an azo dye coupling component and produced by applying to a suitable base a coating solution containing said diazo compound and said azo dye component, which comprises adding to the coating solution a member of the group consisting of saturated and unsaturated gamma lactones of the following formulae:



15 wherein X is a member of the group consisting of H, OH, COOH and alkyl, Y is a member of the group consisting of H and alkyl, Z is a member of the group consisting of H and OH, R is a lower alkyl radical, R1 is a member of the group consisting of H and COOH, and Alk means alkylene; and coating a suitable base with said solution.

20 3. The process of increasing the stability of a diazo-type light-sensitive layer containing a diazo compound derived from a para amino aniline compound and an azo dye coupling component and produced by applying to a suitable base a coating solution containing said diazo compound and said azo dye component, which comprises adding to the coating solution a member of the group consisting of saturated and unsaturated gamma lactones of the following formulae:



45 wherein X is a member of the group consisting of H, OH, COOH and alkyl, Y is a member of the group consisting of H and alkyl, Z is a member of the group consisting of H and OH, R is a lower alkyl radical, R1 is a member of the group consisting of H and COOH, and Alk means alkylene; and coating a suitable base with said solution.

50 4. The process of increasing the stability of a diazo-type light-sensitive layer containing a diazo compound derived from an ortho amino naphthol compound and an azo dye coupling component and produced by applying to a suitable base a coating solution containing said diazo compound and said azo dye component, which comprises

adding to the coating solution a member of the group consisting of saturated and unsaturated gamma lactones of the following formulae:

the group consisting of saturated and unsaturated gamma lactones of the following formulae:



and



wherein X is a member of the group consisting of H, OH, COOH, and alkyl, Y is a member of the group consisting of H and alkyl, Z is a member of the group consisting of H and OH, R is a lower alkyl radical, R<sub>1</sub> is a member of the group consisting of H and COOH, and Alk means alkylene; and coating a suitable base with said solution.

5. The process of increasing the stability of a diazo-type light-sensitive layer containing a diazo compound obtained from an ortho amino naphthol compound and an azo dye coupling component and produced by applying a coating solution containing said diazo compound and azo dye component on a suitable base, which comprises adding gamma valero lactone to the coating solution and coating a suitable base with said solution.

6. The process of increasing the stability of a diazo-type light-sensitive layer containing a diazo compound obtained from a para amino aniline compound and an azo dye coupling component and produced by applying a coating solution containing said diazo compound and azo dye component to a suitable base, which comprises adding gamma valero lactone  $\gamma$  carbonic acid to the coating solution and coating a suitable base with said solution.

7. The process of increasing the stability of a diazo-type light-sensitive layer containing a diazo compound obtained from a para amino aniline compound and an azo dye coupling component and produced by applying a coating solution containing said diazo compound and said azo dye component to a suitable base, which comprises adding the gamma-di-hydroxy lactone of the gamma-hydroxy crotonic acid to the coating solution and coating a suitable base with said solution. 70

8. Light-sensitive layers on a suitable base comprising a diazo compound suitable for forming a stable two component diazo-type layer, an azo dye coupling component and a member of



or and



wherein X is a member of the group consisting of H, OH, COOH and alkyl, Y is a member of the group consisting of H and alkyl, Z is a member of the group consisting of H and OH, R is a lower alkyl radical, R<sub>1</sub> is a member of the group consisting of H and COOH, and Alk means alkylene.

9. Light-sensitive layers on a suitable base comprising a diazo compound obtained from a para amino aniline compound, an azo dye coupling component, and a member of the group consisting of saturated and unsaturated gamma lactones of the following formulae:



65 and



wherein X is a member of the group consisting of H, OH, COOH and alkyl, Y is a member of the group consisting of H and alkyl, Z is a member of

the group consisting of H and OH, R is a lower alkyl radical, R<sub>1</sub> is a member of the group consisting of H and COOH, and Alk means alkylene.

10. Light-sensitive layers on a suitable base comprising a diazo compound obtained from an ortho amino naphthol compound, an azo dye coupling component, and a member of the group consisting of saturated and unsaturated gamma lactones of the following formulae:



and



wherein X is a member of the group consisting of H, OH, COOH and alkyl, Y is a member of the group consisting of H and alkyl, Z is a member of the group consisting of H and OH, R is a lower alkyl radical, R<sub>1</sub> is a member of the group consisting of H and COOH, and Alk means alkylene.

11. Light-sensitive layers on a suitable base comprising a diazo compound obtained from an ortho amino naphthol compound, an azo dye coupling component and gamma valero lactone.

12. Light-sensitive layers on a suitable base comprising a diazo compound obtained from a para amino aniline compound, an azo dye coupling component, and gamma valero lactone  $\gamma$  carbonic acid.

13. Light-sensitive layers on a suitable base comprising a diazo compound obtained from a para amino aniline compound, an azo dye coupling component and the  $\gamma$  di-hydroxy lactone of gamma-hydroxy crotonic acid.

30

MAXIMILIAN K. REICHEL.